

## [54] ROTARY CASTING METHOD OF KILLED STEEL

[76] Inventors: **Kimio Saito; Yutaka Fujisawa**, both of c/o Itoh Iron & Steel Works Co., Ltd., No. 4-1, 5-chome, Matsue, Edogawa-ku, Tokyo, Japan

[22] Filed: May 25, 1971

[21] Appl. No.: 146,674

[52] U.S. Cl. .... 164/126, 164/136

[51] Int. Cl. .... B22d 27/04, B22d 27/08

[58] Field of Search ... 164/114, 118, 122, 126, 128, 164/136, 286, 348

## [56] References Cited

## UNITED STATES PATENTS

448,881 3/1891 Hinsdale ..... 164/122

3,364,978 1/1968 Tanoue et al. .... 164/114

3,414,966 12/1968 Devin et al. .... 164/114 UX

## FOREIGN PATENTS OR APPLICATIONS

1,324,225 3/1963 France ..... 164/114

## OTHER PUBLICATIONS

Making, Shaping, & Treating of Steel, U.S. Steel, 8th Ed., 1964, pp. 548-549.

Primary Examiner—Robert D. Baldwin

Assistant Examiner—John E. Roethel

[57]

## ABSTRACT

A rotary casting method for making a killed steel ingot wherein molten steel is charged into the ingot mold, the charged molten steel on its surface being sprayed with water or compressed cold air to form a coagulation layer, and after passage of a predetermined time period the ingot mold containing the molten steel is inverted or is positioned in horizontal direction, whereafter the inverted or horizontally directed ingot mold is returned to its original vertical upright position for coagulation of the molten steel.

5 Claims, 3 Drawing Figures



PATENTED JAN 22 1974

3,786,855

FIG.1



FIG.2



FIG.3



INVENTOR

KIMIO SAITO, YUTAKA FUJISAWA

BY

ATTORNEY

## ROTARY CASTING METHOD OF KILLED STEEL

## BACK GROUND OF THE INVENTION

In casting methods heretofore practiced, the completely deoxidized liquid steel has been charged into an ingot mold with the formation of a globular shrinkage pipe having an oxidized surface at the center of the steel ingot head, which therefore can not be welded even when subjected to the blooming mill and, as a result, must be cut off with considerably low yield.

In this respect, improvement in yield by avoiding loss resulting from the severing of shrinkage pipe is an important consideration in the art of casting killed steel.

To increase the yield ingot molds have been specially designed with emphasis on charging conditions for the molten steel. It has also been the practice to provide a feeder head on the ingot mold in order to gather the shrinkage pipe therein for subsequent cutting off of the said feeder head section after the rolling step. To initiate coagulation and to prevent oxidation within the pipe it has been the practice to pour water on the ingot steel head.

In the known methods, however, the feeder head is eventually removed and the undesirable oxidation nevertheless results.

## SUMMARY OF THE INVENTION

It is, accordingly, a general object of the invention to obviate the above difficulties and disadvantages and to provide a novel ingot casting method for making a killed steel with improved yield.

In accordance with the present invention, the surface of the liquid steel after being charged into the ingot mold is sprayed with water or with compressed cold air to form a coagulation layer and with rotation of the ingot mold, the pipe resulting from shrinkage during coagulation is dispersed in the forms of the small cavities at along the axis of the resulting ingot thereby preventing undesirable oxidation in the ingot steel.

Another object of the present invention is to provide a rotary casting method for making a killed steel which comprises charging the molten steel into the ingot mold, spraying water or compressed cold air onto the surface of the charged molten steel to form a coagulation layer, inverting the mold for a predetermined time period or alternatively rotating the mold containing the molten steel to be horizontally positioned, whereafter the inverted or horizontally positioned ingot mold is rotated to its original vertical upright position for the completion of coagulation of the molten steel.

The ingot steel obtained by practice of the invention exhibits in section a homogeneous composition having disposed therein a shrinkage pipe in the form of small cavities along the longitudinal axis of the ingot.

Other objects and advantages of the killed steel casting method according to the invention will become apparent from a consideration of the following detailed description taken in conjunction with the accompanying drawings wherein preferred embodiments of the invention are shown. However, it will be understood that the invention is not limited to the details disclosed but includes all such variations and modifications as fall within the spirit of the invention and the scope of the appended claims.

## BRIEF DESCRIPTION OF THE DRAWINGS

In the drawings:

- 5 FIG. 1 is a sectional elevation of the killed ingot steel cast in accordance with the conventional method;
- 10 FIG. 2 is a sectional elevation of the killed ingot steel cast in accordance with the present invention wherein the ingot steel after being charged into the ingot mold is inverted 180°; and
- 15 FIG. 3 is a sectional elevation of the killed ingot steel cast in accordance with the present invention wherein the ingot steel after being charged into the ingot mold is rotated 450° from an upright vertical position to its illustrated horizontal positioned and then returned to its original vertical upright position.

## DETAILED DESCRIPTION OF THE INVENTION:

The method of this invention will be further discussed hereinbelow in conjunction with the accompanying drawings.

In operation, the molten steel which has been completely deoxidized with deoxidizers such as Si, Mn and the like by a known process is charged into the ingot mold. A few minutes after completion of the charging, the exposed surface in the ingot mold is sprayed with water or with compressed cold air to form a coagulation layer thereon. The ingot mold is then reversed and thereafter returned to its original upright vertical position for completing coagulation. Alternatively, the ingot mold after being charged with the molten steel rotated one revolution plus 90° (i.e. 450°) and brought to rest in its horizontal position for 5-10 seconds, whereafter its returned to its original upright vertical position. The ingot mold may be sealed by a cover for prevention of the disadvantageous oxidation and any unexpected accident such as an over-flow of the liquid steel.

The following non-limitative examples, in which all parts are expressed by weight, will serve to illustrate the practice of the invention in more detail.

## EXAMPLE 1

350 Kg of molten steel is poured into the ingot mold for direct casting at an outlet temperature of 1,600°C for a charging time of 38 seconds and after 30 seconds pass, the exposed head surface has poured thereon about 200 cc of water. After the 3 minutes 55 seconds pass from the charging operation, the ingot mold is rotated 180°, which takes 3 minutes, and returned into its original upright vertical position for completion of coagulation.

## EXAMPLE 2

350 Kg of molten steel is poured into the ingot mold for direct casting at an outlet temperature of 1,640°C with a charging time of 43 seconds and 30 seconds thereafter, the exposed head surface has formed thereon about 200 cc of water. After elapse of 3 minutes 20 seconds pass from the charging operation, the ingot mold is rotated one and a quarter turns, i.e., rotated 450°, which takes 3 minutes 30 seconds, and maintained in a horizontal position for 6 seconds and subsequently returned to its original upright vertical position for the coagulation purpose.

Sectional views of steel ingot cast in accordance with the above Examples 1 and 2 are shown in FIGS. 2 and 3. As is apparent from the drawings, no shrinkage pipe

globules are formed at the head and bottom of the ingot. Instead only cavities of small size are dispersed somewhat near the center axis. More particularly, a steel ingot cast according to Example 2, will exhibit colonies of cavities dispersed about the center axis, said cavities being completely isolated by the environmental chill crystal zone forming the outer contour of the ingot, whereby undesirable oxidation is prevented.

In accordance with the killed steel cast by the present invention, no oxidized layer is formed on the inner surface thereof despite the presence of small pipe colonies dispersed therein. Moreover these pipes may be eliminated by subjecting them to squeezing pressure during the rolling operation without need therefore for cutting away sections as in prior art thereby increasing the yield considerably.

As a result of the fracture tests of the ingot steel cast in accordance with the present invention by, for example, the S print test or the macroscopic corrosion test, no remarkable segregation could be seen and hence an ingot steel of homogeneous composition has resulted with an improved yield.

What we claim are:

1. A method of casting a steel ingot, which comprises charging molten steel into a vertically arranged ingot mold, chilling the exposed surface of the charged molten steel to form a coagulation layer, rotating the ingot

5 mold through at least 180° about a horizontal axis during a time sufficient to disperse the resulting shrinkage pipe in the form of small cavities along the axis of the resulting ingot, maintaining the ingot mold in its rotated position for a time sufficient to stabilize the resulting small-cavity pipe dispersion, and thereafter returning the ingot mold to a vertical position.

10 2. A method according to claim 1, wherein the ingot mold after being charged with molten steel is rotated 180° for a predetermined time, whereafter the ingot mold is rotated to its original vertical position.

15 3. A method according to claim 1, wherein the ingot mold after being charged with molten steel is rotated 450° from its upright vertical position for a predetermined period for disposition in a horizontal direction, maintaining the ingot mold in said horizontal direction for a predetermined time, and returning, after said lapse of said predetermined time, said ingot mold to its original position.

20 4. A method according to claim 3, wherein said ingot mold is maintained in said horizontal position for between 5 to 10 seconds.

25 5. A method according to claim 3, wherein said ingot mold is maintained in said horizontal direction for 6 seconds.

\* \* \* \* \*

30

35

40

45

50

55

60

65